

# UNITED STATES PATENT OFFICE.

EDWARD F. MILLARD, OF HOPKINTON, MASSACHUSETTS.

## PROCESS OF MAKING WOOD PULP.

1,413,180.

Specification of Letters Patent. Patented Apr. 18, 1922.

No Drawing.

Application filed June 7, 1921. Serial No. 475,775.

To all whom it may concern:  
Be it known that I, EDWARD F. MILLARD, citizen of the United States, residing at Hopkinton, in the county of Middlesex and 5 State of Massachusetts, have invented certain new and useful Improvements in Processes of Making Wood Pulp, of which the following is a specification, reference being had therein to the accompanying drawing.

My present invention relates to an improved process of making wood pulp, and has for its principal object the reduction of pressure to the wood stock and the elimination of the use of hard grindstones.

In making wood pulp it has previously been the custom to place the wood stock in a cylinder or other suitable receptacle and subject it to a high pressure whereby it is forced against a grinding stone which is rotated to remove the fibre, the grindstones used being of hard material to withstand the pressure. Only hard grindstones have been employed and the pressure has been adapted 20 to the condition of the stone whether sharp or worn and smooth, and a relatively light pressure has been employed in connection with a sharp stone. Such grindstones when first dressed produce a large proportion of 25 slivers and short thick particles, which weakens the pulp. As the stone wears smooth, a better pulp is produced, but a large quantity of wood flour is made, which goes to waste, also cutting down the production.

In carrying out my present process I propose to place the wood stock in the usual form of machine, such as illustrated in my Patent No. 780,213, dated January 17, 1905, 30 having a cylinder or other form of receptacle therefor, but instead of using high pressure to force the stock against the grindstone, I will use the minimum amount of pressure necessary to cause the stock to frictionally engage the grindstone which will be of relatively soft material such as sandstone, or manufactured stone having a soft bond. I refer to the minimum pressure

explained in the aforesaid patent, namely a relatively light pressure, that is to say 50 approximately 3500 lbs., which is approximately one-third of what is commonly used in heavy pressure machines. By a soft grindstone I mean a grindstone in which the grit is held loosely adherent by a soft 55 bond. A stone of this character will not take a polish or wear smooth, has a surface of the desired roughness (the nature and quality of the surface not being affected as the elements wear), and produces fine and 60 long fibres which are uniform. The stone will give off particles on its active periphery to maintain the substantially constant and uniform frictional engagement between the stone and wood stock, thus eliminating 65 excessive pressure as well as minimizing drive power. For making short fibres a fine grit stone is necessary, whereas to produce long fibres a coarse grit stone is preferable. It is hardly possible to get these 70 natural sandstones of both fine and coarse grit, and for this reason it is necessary to dress the stone to get both fine and coarse grit results. On the other hand, if desired, manufactured stone having a soft bond may 75 be used.

Having described my invention, what I claim as new and desire to secure by Letters Patent, is:

The method of producing uniform mechanical fibre from raw wood without flour or coarse particles, which consists in presenting wood to a grinding surface of grit and soft bond such that it would be substantially effaced under the usual grinding 80 pressure and applying to such wood and grinding surface a pressure so light that it would not substantially efface said soft grinding surface.

In testimony whereof I hereunto affix my 90 signature in the presence of two witnesses.

EDWARD F. MILLARD.

Witnesses:

ERNEST H. ADAMS,  
ALBERT B. C. DEMING, Jr.